

UNITED STATES PATENT OFFICE.

TENNEY L. DAVIS, OF SOMERVILLE, MASSACHUSETTS.

## PROCESS FOR PRODUCING SMOKELESS POWDER.

No Drawing.

Application filed April 16, 1921. Serial No. 462,028.

(FILED UNDER THE ACT OF MARCH 3, 1883, 22 STAT. L., 625.)

*To all whom it may concern:*

Be it known that I, TENNEY L. DAVIS, a citizen of the United States, and a resident of Somerville, county of Middlesex, and State of Massachusetts, have invented an Improvement in Processes for Producing Smokeless Powder, of which the following is a specification.

The invention described herein may be

55

rendering the surface less pervious to moisture and slower burning than the surfaces of uncoated powder grains. Incorporated throughout the mass of powder grain, these substances render the powder slower burning and cooler, and consequently reduce its erosive effect and, in certain cases, may even produce flashlessness of discharge.

The invention described herein may be used by the Government, or any of its officers or employees in prosecution of work for the Government, or by any other person in the United States, without payment to me of any royalty thereon.

15 The subject of this invention is "Gelatinizing agents for nitrocellulose." The main advantages of this invention reside in the fact that powders coated with the substances will be less hygroscopic than 20 ordinary smokeless powder and will show in a greater degree the phenomenon of "progressive burning," giving higher velocity to the projectile while producing lower gas pressures in the barrel of the gun.

25 Whether these substances are incorporated throughout the mass of powder grain or are only amalgamated with the surface they will have the effect of rendering the powder cooler and slower. As these substances are  
30 not sensibly hygroscopic, their use in place of part or all of the usual alcohol-ether or acetone solvent, will reduce the tendency of the powder to take moisture. Their amount may be so regulated as to render the powder  
35 flashless.

For some time it has been the practice to incorporate with the nitrocellulose which is used in the manufacture of smokeless powder certain other nitrogenous substances, 40 particularly substituted ureas and substituted urethanes which modify the nature of the resulting colloid. Certain of these substances act also as "stabilizers," combining with the products of the spontaneous 45 decomposition of the nitrocellulose and so lengthening the effective life of the powder. These same substances are used also for coating smokeless powder grains. When applied to powder by methods which are 50 well known, these substances amalgamate with the surface of the grain and modify its

physical condition rendering the surface less pervious to moisture and slower burning than the surfaces of uncoated powder grains. Incorporated throughout the mass of powder grain, these substances render the powder slower burning and cooler, and consequently reduce its erosive effect and, in certain cases, may even produce flashlessness of discharge. 55

I have discovered that certain nitrogen compounds of the type known as "heterocyclic" compounds are excellent solvents for nitrocellulose and eminently satisfactory for use as gelatinizing agents in the manufacture of smokeless powder and for use in coating grains of nitrocellulose powder. Noteworthy among such substances are the substituted pyrazolones and pyrazolidones. The formulas of the unsubstituted parent substances are given below:



My experiments indicate for instance, that 75 diphenylpyrazolone is about three times as efficient a gelatinizer for nitrocellulose as other standard gelatinizing agents with which I have compared these substances. I 80 find that phenyldimethylpyrazolone, which has been used extensively in medicine under the name of "antipyrine" is also an excellent material for the purpose.

What I claim as new and desire to secure by Letters Patent, is:

1. A process for producing smokeless powder, embodying gelatinizing nitrocellulose with a nitrogen compound of the heterocyclic type, forming the colloid thus obtained into grains and drying. 90

2. A process for producing smokeless powder embodying gelatinizing nitrocellulose with a substituted pyrazolone derivative, forming the colloid thus obtained into grains and drying. 95

3. A process for producing smokeless powder, embodying gelatinizing nitrocellulose with a substituted pyrazolidone, forming the colloid thus obtained into grains and drying.

TENNEY L. DAVIS.